

## 1

3,379,550

 PARAFFIN-MICROCRYSTALLINE WAX  
COMPOSITION

John Podlipnik, Palos Heights, Ill., assignor to Sinclair Research, Inc., New York, N.Y., a corporation of Delaware  
No Drawing. Filed June 26, 1964, Ser. No. 378,449  
5 Claims. (Cl. 106—270)

This invention relates to wax compositions for coating of paper and paperboard cups and other containers. The compositions impart a high degree of rigidity to the container along with a smooth, non-glossy, satin-like finish.

Petroleum waxes are used extensively for coating of paper and paperboard cups used in the dispensing of soft drinks, ice cream sodas and malts, etc. Among other things, the wax serves to strengthen and waterproof the cup. The strength is of particular importance in dispensing of ice cream sodas and malts since in many cases the cup serves to hold the contents during blending, and the nature of the contents is such that any loss in strength due to penetration of water into the board is undesirable. The wax should be such as to result in a smooth, continuous, satin-like finish. In addition, the melting point and blocking temperature of the coating should be sufficiently high to prevent sticking of the wax-coated cups when they are nested.

Many of the waxes presently used as cup coatings fail to provide a high degree of strength along with a smooth finish. Attempts to improve smoothness and strength through the use of polymers such as polyethylene and various resins have been unsuccessful. While such additives provide smooth continuous coatings they do not give the desired rigidity, and, in fact, they many times adversely affect rigidity. Furthermore, they are costly and increase viscosity which adversely affects machine performance.

It has now been found that by blending a certain narrow range approximately 138–145° F. melting point paraffin wax with about 5 to 10% by weight of a particular microcrystalline wax, a paper and paperboard cup coating composition is produced which provides outstanding rigidity and excellent cup appearance.

The paraffin wax should be a relatively narrow range material composed of essentially straight chain paraffins. It should have the following approximate properties:

|                                            |             |
|--------------------------------------------|-------------|
| Melting point, ° F. ASTM D-87              | 138–145     |
| Viscosity at 210° F., SSU                  | 38–42       |
| Penetration at 77° F. ASTM (D-1321)        | 7–11        |
| Refractive index at 80° C.                 | 1.429–1.432 |
| 10–90% distillation range at 760 mm., ° F. | 700–950     |

By the 10 to 90% distillation range it is meant that the actual 10 to 90% distillation range of the wax is within the range of about 700 to 950° F., preferably within about 725 to 925° F., often with a 10 to 90% spread of about 100 to 225° F. unit within the ranges cited. The paraffin wax can be prepared by conventional phenol extraction, methyl ethyl ketone dewaxing, and methyl ethyl ketone deoiling of a waxy petroleum distillate having an appropriate distillation range.

Paraffin waxes whose properties fall outside of these ranges are unsatisfactory. For example, if the viscosity is above about 42 SSU at 210° F., this leads to difficulties in machine performance and higher wax consumption. Waxes with melting points below about 138° F. generally have too low blocking points for this application. Broad range waxes having wider distillation ranges do not provide desired rigidity and adversely affect machine performance. Tests on a blend in which a broad range wax

## 2

composed of 127/129° F., 142/144° F., and 152/154° F. melting point waxes (overall 10–90% distillation range of 680° F.–1000° F.) was used, showed such a blend to lack sufficient rigidity.

Also, difficulty was experienced with wax buildup on machine parts. The preferred paraffin wax has a melting point of about 142 to 144° F.

The microcrystalline wax of the present invention should have the following approximate properties:

|                                               |         |
|-----------------------------------------------|---------|
| Melting point, ° F. ASTM D-127                | 180–200 |
| Penetration at 77° F., 100 gms. ASTM (D-1321) | 2–8     |
| Viscosity at 210° F., SSU                     | 60–90   |

Microcrystalline waxes which meet these requirements can be used as the minor constituent of the wax composition. The microwax preferably can be a tank bottom microcrystalline wax which is the high melting point wax obtained by the refining of the waxy materials which settle out of crude oil during storage or the high melting point microcrystalline waxes in this range prepared by the conventional solvent deoiling of petrolatum. The properties and the concentration of the microcrystalline wax blended with the paraffin wax component are important. Microwaxes which do not meet the required properties fail to provide the desired satin-like coating and rigidity. Employment of less than about 5% of the microcrystalline wax also fails to give the desired smooth, non-glossy coating. Use of greater than about 10% by weight of the microcrystalline wax tends to embrittle the wax and provides a final blend which leads to excessive build up on machine parts, high wax consumption, and possible difficulties with settling of microwax in storage tanks. The preferred microwaxes are the tank bottom microcrystalline waxes having a melting point of about 190 to 195° F. (ASTM D-127) and when blended with the preferred paraffin wax, i.e. of about 142/144° F., melting point, may, with advantage be added in an amount of about 6% by weight. The wax blends of the invention have the following approximate properties:

|                                | Typical | Range        |
|--------------------------------|---------|--------------|
| Melting Point, ° F., ASTM D-87 | 143     | 138–146      |
| Viscosity at 210° F., SSU      | 42      | 41–44        |
| Penetration at 77° F.          | 8       | 6–11         |
| Refractive Index at 80° C.     | 1.4310  | 1.4290–1.432 |
| Cloud Point, ° F.              | 159     | 155–165      |

Without the defined paraffin wax and microcrystalline waxes and in the defined proportions these properties are not met.

Although the wax of the present invention exhibits its greatest advantage with respect to the coating of paper and paperboard cup or similar containers, it can be used as well in the coating of other paper and paperboard articles.

The following example is included to further illustrate the present invention.

60 Example

Several waxes and wax blends identified in the table below were used to coat paper cups in the laboratory and on commercial equipment.

65 The procedure used in the laboratory to coat the sample cups consisted of immersing tared 16 oz. cups in the wax sample at 205° F. for 15 seconds followed by draining and solidification in room temperature air. During draining the cup is held upside down until the coating solidifies. Consumption is determined by weighing the waxed cups and determining wax pickup.

Commercial coatings were also performed on a spray coating machine in which the wax is sprayed at about 200° F. on a cup rotating on a spindle. The sprayed cup rides upside down through a heat tunnel after which it is cooled with room temperature air.

All of the coated cups were evaluated as to appearance and several coated cups were subjected to a crush test. An uncoated cup was also tested for comparison. Two crush tests were employed, the vacuum crush test and the Squashometer test.

In the vacuum crush test the wax cup is placed upside down on the center neck of a three necked flask, and the lip of the cup sealed to the flask using silicone grease. Vacuum is applied to the flask and the cup at a constant rate of evacuation, and the reduction in pressure measured with a manometer containing  $CCl_4$ . At a certain point the cup is unable to withstand outside air pressure and collapses breaking the vacuum. The manometer reading is measured and recorded as the vacuum crush value in centimeters of  $CCl_4$ .

The Squashometer test consists of applying a force at a constant rate at two diametrically opposite points of the cup about 2% inches from the bottom of the 16 oz. cup. The total force required to crush the cup is measured and called the Squashometer value.

The waxes and wax compositions evaluated and the test results are summarized in the table:

A comparison of blend 1 with blends 2 and 3 and a comparison of blend 6 with blend 7 show the need to add at least 5% of a 180-200° F. melting point microcrystalline wax to obtain a smooth, satin, non-glossy appearance. The high rigidity (as measured by the force required to crush the cups) provided by the narrow melting point range paraffin wax of the invention is shown by comparing blends 3 and 4 with blend 7. Note that the melting point and other physical properties of blend 7 were almost identical to those of blend 4, yet the rigidity provided by blend 7 was unacceptable. It appears from these results that it is the presence of the low melting, relatively low boiling 129° F. melting point and high melting point waxes that lead to less rigidity with blend 7.

It is claimed:

1. A wax composition consisting essentially of a straight chain paraffin wax having a melting point (ASTM D-87) of about 138 to 145° F.; a viscosity at 210° F. of about 38 to 42 SSU; a penetration at 77° F. (ASTM D-1321) of about 7 to 11; a refractive index at 80° C. of about 1.429 to 1.432 and a 10-90% distillation range at 760 mm. in the range of about 700 to 950° F., and about 5 to 10% by weight of a microcrystalline wax having a melting point (ASTM D-127) of about 180 to 200° F.; a penetration at 77° F. (ASTM D-1321) of about 2 to 8 and a viscosity at 210° F. of about 60 to 90 SSU.

TABLE.—PROPERTIES OF PAPER CUPS COATED WITH VARIOUS WAXES

| Wax Identity                               | 1             | 2               | 3             | 4             | 5             |
|--------------------------------------------|---------------|-----------------|---------------|---------------|---------------|
| <b>Base Waxes:</b>                         |               |                 |               |               |               |
| 129° F. M.P. Paraffin Wax                  |               |                 |               |               |               |
| 143° F. M.P. Paraffin Wax                  | 100           | 96              | 95            | 94            | 93            |
| 153° F. M.P. Paraffin Wax                  |               |                 |               |               |               |
| 194° F. M.P. Tank Bottoms Microwax         |               | 4               | 5             | 6             | 7             |
| <b>Laboratory Coated 16 oz. Cups:</b>      |               |                 |               |               |               |
| Consumption, Lbs./1,000 cups               |               |                 | 12.1          |               | 11.2          |
| Vacuum Crush cm. of $CCl_4$                |               |                 | 55            | 60            | 55            |
| <b>Appearance:</b>                         |               |                 |               |               |               |
| Gloss                                      | Some gloss    | Very slight     | None          | None          | None          |
| Orange Peel                                | Pronounced    | Slight          | do            | do            | do            |
| Feel                                       | Rough, grainy | Slightly grainy | Smooth, satin | Smooth, satin | Smooth, satin |
| <b>Commercially Coated 16 oz. Cups:</b>    |               |                 |               |               |               |
| Consumption, Lbs./1,000 cups               |               |                 |               | 11.3          |               |
| Squashometer Crush, Grams                  |               |                 |               | 1,525         |               |
| <b>Appearance:</b>                         |               |                 |               |               |               |
| Gloss                                      |               |                 | None          |               |               |
| Orange Peel                                |               |                 | do            |               |               |
| Feel                                       |               |                 | Smooth, satin |               |               |
| <b>Physical Properties:</b>                |               |                 |               |               |               |
| Melting Point, ° F. ASTM D-87              | 143.5         |                 |               | 143.2         |               |
| Melting Point, ° F. ASTM D-127             |               |                 |               |               |               |
| Viscosity at 210° F., SUS                  | 40.7          |                 |               | 41.8          |               |
| Penetration at 77° F.                      | 8             |                 |               | 8             |               |
| Refractive Index at 80° C.                 | 1.4309        |                 |               |               |               |
| 10-90% Distillation Range at 760 mm., ° F. | 725-925       |                 |               |               |               |

| Wax Identity                               | 6              | 7             | 8             | 9    | Unwaxed Cup |
|--------------------------------------------|----------------|---------------|---------------|------|-------------|
| <b>Base Waxes:</b>                         |                |               |               |      |             |
| 129° F. M.P. Paraffin Wax                  | 20             | 19            |               |      |             |
| 143° F. M.P. Paraffin Wax                  | 45             | 43            |               |      |             |
| 153° F. M.P. Paraffin Wax                  | 35             | 33            | 100           |      |             |
| 194° F. M.P. Tank Bottoms Microwax         |                | 5             |               | 100  |             |
| <b>Laboratory Coated 16 oz. Cups:</b>      |                |               |               |      |             |
| Consumption, Lbs./1,000 cups               |                | 12.1          |               |      |             |
| Vacuum Crush, cm. of $CCl_4$               |                | 48            |               |      | 22          |
| <b>Appearance:</b>                         |                |               |               |      |             |
| Gloss                                      | Very slight    | None          | Some gloss    |      |             |
| Orange Peel                                | Moderate       | do            | Pronounced    |      |             |
| Feel                                       | Slightly rough | Smooth, satin | Rough, grainy |      |             |
| <b>Commercially Coated 16 oz. Cups:</b>    |                |               |               |      |             |
| Consumption, Lbs./1,000 cups               |                | 10.9-11.1     |               |      |             |
| Squashometer Crush, Grams                  |                | 1,300-1,400   |               |      |             |
| <b>Appearance:</b>                         |                |               |               |      |             |
| Gloss                                      | None           |               |               |      |             |
| Orange Peel                                | do             |               |               |      |             |
| Feel                                       | Smooth, satin  |               |               |      |             |
| <b>Physical Properties:</b>                |                |               |               |      |             |
| Melting Point, ° F. ASTM D-87              | 143            | 143           | 153           |      |             |
| Melting Point, ° F. ASTM D-127             |                |               |               | 104  |             |
| Viscosity at 210° F., SUS                  | 41.7           | 42.1          | 47.4          | 77.0 |             |
| Penetration at 77° F.                      | 10             | 8             | 13            | 3    |             |
| Refractive Index at 80° C.                 | 1.4319         | 1.4320        | 1.4364        |      |             |
| 10-90% Distillation Range at 760 mm., ° F. | 680-1,000      |               | 800-1,000     |      |             |

\*Cups coated at 205° F., 15 seconds dip in wax bath, cooled in room temperature air.

2. The composition of claim 1 wherein the paraffin wax has a melting point of about 142° to 144° F. and the microcrystalline wax is a tank bottom microcrystalline wax having a melting point of about 190 to 195° F.
3. The composition of claim 2 wherein the tank bottom microcrystalline wax is present in an amount of about 6% by weight.
4. A paper cup coated with the composition of claim 1.
5. A paper cup coated with the composition of claim 2.

## References Cited

## UNITED STATES PATENTS

|           |        |           |       |         |
|-----------|--------|-----------|-------|---------|
| 2,773,812 | 5/1954 | Tench     | ----- | 106—270 |
| 2,885,340 | 5/1959 | Tench     | ----- | 208—21  |
| 3,128,241 | 4/1964 | Podlipnik | ----- | 208—21  |

ALEXANDER H. BRODMERKEL, *Primary Examiner.*  
T. MORRIS, *Assistant Examiner.*